

# UNITED STATES PATENT OFFICE.

OTTO BONHOEFFER, OF ELBERFELD, AND HUGO GUNTRUM, OF VOHWINKEL, NEAR ELBERFELD, GERMANY, ASSIGNEES TO FARBEFABRIKEN VORM. FRIEDR. BAYER & CO., OF ELBERFELD, GERMANY, A CORPORATION OF GERMANY.

## CELLULOSE FORMATES AND PROCESS OF MAKING SAME.

1,093,247.

Specification of Letters Patent. Patented Apr. 14, 1914.

No Drawing.

Application filed October 27, 1910. Serial No. 589,449.

To all whom it may concern:

Be it known that we, OTTO BONHOEFFER and HUGO GUNTRUM, doctors of philosophy, chemists, citizens of the German Empire, residing at, respectively, Elberfeld and Vohwinkel, near Elberfeld, Germany, have invented new and useful Improvements in Cellulose Formates and Processes of Making Same, of which the following is a specification.

Our invention relates to the production of formyl derivatives of cellulose (cellulose formates). The process for preparing these new compounds consists in treating a cellulose compound, especially cellulose, hydrocellulose or oxycellulose with formic acid and sulfuryl chlorid or chlorosulfonic acid

20



The process can be promoted by the addition of zinc chlorid.

In carrying out the new process practically we can proceed as follows, the parts being by weight: 20 parts of cotton are introduced into a mixture of 100 parts of formic acid (95 per cent.), 5 parts  $\text{ZnCl}_2$  and 10 parts of sulfuryl chlorid ( $\text{SO}_2\text{Cl}_2$ ). The mixture is well stirred and is allowed to stand for 5-6 hours. The clear thick solution thus obtained is then poured into water, by which means the new formyl cel-

lose being most probably a mixture of different formyl cellulose is separated. It is a whitish voluminous mass soluble in formic acid, in a solution of  $\text{ZnCl}_2$  and is distinguished from the formylcellulose compounds of the old arts by being more soluble in pyridin. On evaporating the solutions of the new formyl celluloses a colorless and translucent flexible film remains.

We claim:

1. The process of producing cellulose esters of fatty acids, which consists in treating cellulose compounds with a reagent containing the radial of a fatty acid in presence of a chlorin derivative of sulfuric acid, substantially as and for the purpose specified.

2. The process of producing the formic acid ester of cellulose, which consists in treating cellulose with formic acid in presence of a chlorin derivative of sulfuric acid, substantially as and for the purpose specified.

In testimony whereof we have hereunto set our hands in the presence of two subscribing witnesses.

OTTO BONHOEFFER. [L. S.]  
HUGO GUNTRUM. [L. S.]

Witnesses:

CHAS. J. WRIGHT,  
ALFRED HENKEL.